

## UNITED STATES PATENT OFFICE.

LEO UBBELOHDE, OF KARLSRUHE, BADEN, GERMANY.

## PROCESS OF MANUFACTURING SPINNING FIBERS.

No Drawing.

Application filed August 2, 1922. Serial No. 579,307.

*To all whom it may concern:*

Be it known that I, LEO UBBELOHDE, a citizen of Germany, residing at Karlsruhe, Baden, whose post-office address is Wendtstrasse 11, Karlsruhe, Baden, Germany, have invented certain new and useful Processes of Manufacturing Spinning Fibers, of which the following is a specification.

This invention has reference to fibers for spinning purposes and to a process of obtaining the same, and it is particularly intended to improve the conditions and process of manufacture of such fibers. There is a great number of fibers possessing very deficient structure for spinning purposes, that is to say of fibers which are either too short, or not properly twisted or are unbroken or not sufficiently roughened to yield a sufficiently durable fleece and a sufficiently durable slubbing and yarn in the spinning process. Such fibers are not well adapted for spinning purposes, even when in admixture with other fibers.

Of fibers of this kind I may mention by way of example wood pulp, cottonized flax fibers and similar products. My invention is intended to better adapt such fibrous material for spinning purposes by providing a roughening of the surface combined with a breaking and twisting of the fibers. This object is accomplished by treating the fibers in the wet or dry condition, and by means of suitable agitating, grinding and centrifugal means with hard, chip-like sharp edged material the longitudinal extension of which is greatly below the length of the fibers themselves, such as glass powder, carborundum powder, infusorial earth and the like. The treatment may for instance be effected in centrifugal mills, carding and opening means and the like. By means of the sharp edges of the granules of the material the fibers are broken and twisted and are superficially roughened. After the treatment the sharp edged material may be eliminated and may be used over again.

It has also been ascertained that in the case of particularly rapid beating machines the action is greatly assisted and increased by employing a partial or complete vacuum,

because under the action of the vacuum the impinging of the fibers against the parts of machinery and the striking of the sharp edged material against the fibers is more intense and more violent. It is therefore preferable to work the process at low pressure or in the vacuum.

My invention may be carried out in various ways and by the use of a great variety of different pieces of apparatus and methods, and it is susceptible of alterations and modifications to conform to existing conditions, and to better adapt it to the requirements of manufacture and to the convenience of the operator, and without deviating from the spirit of my invention the scope of which is defined by the claims as hereunto appended.

I claim:

1. The process of increasing the spinning qualities of vegetable fibers of inferior spinning qualities which consists in treating said fibers for some time with hard chip-like sharp edged granular powdered material the extension of which in the longitudinal direction is far below the length of the fibers, and then removing such material from the fibers.

2. The process of increasing the spinning qualities of wood pulp, cottonized fibers from linen straw, flax, hemp and other fibers of inferior spinning qualities, which consists in treating such fibers with mineral sharp edged, substantially finely granular material.

3. The process of increasing the spinning properties of fibers of comparatively inferior spinning qualities which consists in treating said fibers under reduced pressure with sharp edged finely granular material of a size greatly below the length of said fibers, and then removing said material from said fibers.

4. The process of increasing the spinning qualities of fibrous material, which consists in treating such material with sharp edged granulated chip-like material, and then separating the different kinds of material from each other.

5. The process of treating vegetable fibers of inferior spinning qualities, which con-

sists in treating said material with sharp edged glass powder.

6. The process of treating vegetable fibers of inferior spinning qualities, which consists in treating said fibers with sharp edged glass powder under reduced pressure.

7. As a new article of manufacture superficially roughened spinning fibers produced

by treatment with chip-like, hard granulated material.

8. Vegetable artificially roughened spinning material consisting of fibers artificially roughened by treatment with sharp edged finely granular material.

In testimony whereof I affix my signature.  
LEO UBBELOHDE.